

April 13, 1926.

1,580,921

A. SCHERER

METHOD OF ORNAMENTING ARTICLES

Filed Feb. 10, 1925



*Fig. 1.*



*Fig. 2.*



*Fig. 3.*



*Fig. 4.*

WITNESSES:

*Virgil L. Mares*  
*George A. Gruss*

INVENTOR

*Adolph Scherer*  
BY  
*Joshua R. Torts*  
115 ATTORNEY

## UNITED STATES PATENT OFFICE.

ADOLPH SCHERER, OF PHILADELPHIA, PENNSYLVANIA.

## METHOD OF ORNAMENTING ARTICLES.

Application filed February 10, 1925. Serial No. 8,105.

*To all whom it may concern:*

Be it known that I, ADOLPH SCHERER, a citizen of the United States, residing at Philadelphia, in the county of Philadelphia and State of Pennsylvania, have invented certain new and useful Improvements in Methods of Ornamenting Articles, of which the following is a specification.

My invention relates to methods of ornamenting articles, such as lamp shades, vases and the like.

The objects are to provide a method by which articles may be ornamented with designs of different colors having glass crystals in cluster-like form thereon which stand out in relief on the surface of the article, and by which designs having clean and definite lines may be produced.

These objects, and other advantageous ends which will be described hereinafter, I attain in the following manner, reference being had to the accompanying drawings in which—

Figure 1 is a fragmentary face view of an article ornamented in accordance with the first step of my method,

Figure 2 a like-view, illustrating another step,

Figure 3 a view like Figure 2, illustrating a third step, and

Figure 4 an enlarged fragmentary section through the article and ornamentation thereon.

The surface 1 of an article 2, which may be of parchment, fabric or glass, is coated with a quick drying varnish 3, preferably opaque such as black lacquer, or equivalent material such as collodion or a celluloid solution. After the coating of varnish is dry, a suitable design 4, as of a bird, is painted, preferably through a stencil, on the coating, with a colored varnish solvent or thinner, or a paint having the solvent therein, to soften the varnish coating. Glass crystals 5, commonly known as beads, are strewn over the design. The glass crystals are caused to sink through the paint and softened varnish to the surface of the article. The crystals as they are strewn, accumulate in cluster-like form and stand out in relief on the surface. The paint and softened varnish with the clustered crystals embedded therein are then allowed to dry, after which the orna-

mented surface is coated with a clear varnish to protect it from moisture. The product is a rich ornamentation of various colors having clean and definite lines.

If the article is transparent or translucent, such as a lamp shade, the light passing through the article will pass through the glass crystals contacting therewith and illuminate the various colors of the dried solvents in which the crystals are embedded. The opaque varnish coating on the article will prevent light from passing through the shade, and thus give the design clean and definite lines.

Ornamentation by this method does not require highly skilled labor and the article produced is rich in appearance and will withstand rough usage, such as received in shipping and handling.

While I have described my invention as taking a particular form, it will be understood that the various parts may be changed without departing from the spirit thereof, and hence I do not limit myself to the precise construction set forth, but consider that I am at liberty to make such changes and alterations as fairly come within the scope of the appended claims.

Having thus described my invention, what I claim as new and desire to secure by Letters Patent is:—

1. The herein described method of ornamenting articles, consisting of coating the article with a quick drying material; painting a design on the dried material with a colored solvent to soften the same, and applying crystals to the colored solvent and softened material.

2. The herein described method of ornamenting articles, consisting of coating the article with a quick drying material, painting a design on the dried material with a colored solvent to soften the same, applying crystals to the solvent and softened material, and causing the crystals to sink through the solvent and softened material to contact with the article.

3. The herein described method of ornamenting articles consisting of coating the article with an opaque quick drying material, painting a design on the dried material with a colored solvent to soften the same, applying crystals to the solvent and

55

60

65

70

75

80

85

90

95

100

105

softened material, and causing the crystals to sink through the design and softened material to contact with the article.

4. The herein described method of ornamenting articles consisting of coating the article with a quick drying varnish, painting a design on the dried varnish with a colored varnish solvent to soften the same, and applying crystals to the solvent and 10 softened varnish.

5. The herein described method of ornamenting articles consisting of coating the article with an opaque lacquer, painting a design on the lacquer with a colored lacquer solvent to soften the same, and applying crystals to the solvent and softened lac- 15

quer and causing the crystals to sink through the design and lacquer to contact with the article.

6. The herein described method of ornamenting articles, consisting of coating the articles with a quick drying material, painting a design on the dried material with a colored solvent to soften the same, applying crystals to the solvent and softened material, drying the solvent and softened material, and applying a protecting coating to the dried material and crystals. 20 25

In testimony whereof I have signed my name to this specification.

ADOLPH SCHERER.